



US005846680A

# United States Patent [19]

Adachi et al.

[11] Patent Number: 5,846,680

[45] Date of Patent: Dec. 8, 1998

- [54] **ELECTROPHOTOGRAPHIC  
PHOTOCONDUCTOR AND AROMATIC  
POLYCARBONATE RESIN FOR USE  
THEREIN**

[75] Inventors: **Chihaya Adachi**, Ueda; **Masaomi Sasaki**, Susono; **Kazukiyo Nagai**, Numazu; **Tomoyuki Shimada**, Shizuoka-ken; **Chiaki Tanaka**, Shizuoka-ken; **Nozomu Tamoto**, Shizuoka-ken; **Akira Katayama**, Shizuoka-ken; **Mitsutoshi Anzai**, Kawasaki; **Akihiro Imai**, Kawasaki; **Katsuhiro Morooka**, Kawasaki, all of Japan

[73] Assignees: **Ricoh Company, Ltd.**, Tokyo; **Hodogaya Chemical Co., Ltd.**, Kawasaki, both of Japan

[21] Appl. No.: **770,684**

[22] Filed: **Dec. 19, 1996**

[30] **Foreign Application Priority Data**

|               |      |       |       |         |
|---------------|------|-------|-------|---------|
| Dec. 19, 1995 | [JP] | Japan | ..... | 7-33047 |
| Jan. 23, 1996 | [JP] | Japan | ..... | 8-00940 |
| Jan. 30, 1996 | [JP] | Japan | ..... | 8-01409 |
| Dec. 16, 1996 | [JP] | Japan | ..... | 8-33600 |
| Dec. 18, 1996 | [JP] | Japan | ..... | 8-33829 |

[51] Int. Cl.<sup>6</sup> ..... **G03G 5/00**

[52] U.S. Cl. ..... **430/73**; 430/59; 430/8

[58] Field of Search ..... **430/73, 59, 8**

[56] **References Cited**

## U.S. PATENT DOCUMENTS

- |           |        |                        |        |
|-----------|--------|------------------------|--------|
| 5,486,439 | 1/1996 | Sakakibara et al. .... | 430/83 |
| 5,547,792 | 8/1996 | Shimada et al. ....    | 430/73 |
| 5,604,064 | 2/1997 | Nukada et al. ....     | 430/59 |
| 5,639,581 | 6/1997 | Iwasaki et al. ....    | 430/59 |

5,736,285 4/1998 Nukada et al. .... 430/83

*Primary Examiner*—Roland Martin  
*Attorney, Agent, or Firm*—Oblon, Spivak, McClelland,  
Maier & Neustadt, P.C.

[57]

## ABSTRACT

An electrophotographic photoconductor includes an electro-conductive support, and a photoconductive layer formed thereon containing as an effective component an aromatic polycarbonate resin having a repeat unit of formula (I), or two repeat units of formulae (II) and (III):



wherein Ar<sup>1</sup> to Ar<sup>6</sup>, X, n, k and j are as specified in the specification.

**22 Claims, 10 Drawing Sheets**



F I G. 1



F I G. 2



F I G. 3



F I G. 4



FIG. 5



FIG. 6



FIG. 7



FIG. 8



FIG. 9



FIG. 10



FIG. II



FIG. 12



FIG. 13



FIG. 14



**ELECTROPHOTOGRAPHIC  
PHOTOCONDUCTOR AND AROMATIC  
POLYCARBONATE RESIN FOR USE  
THEREIN**

**BACKGROUND OF THE INVENTION**

**1. Field of the Invention**

The present invention relates to an electrophotographic photoconductor comprising an electroconductive support, and a photoconductive layer formed thereon, comprising an aromatic polycarbonate resin as an effective component. In addition, the present invention also relates to the above-mentioned aromatic polycarbonate resin with charge transporting properties.

**2. Discussion of Background**

Recently organic photoconductors are used in many copying machines and printers. These organic photoconductors have a layered structure comprising a charge generation layer (CGL) and a charge transport layer (CTL) which are successively overlaid on an electroconductive support. The charge transport layer (CTL) is a film-shaped layer comprising a binder resin and a low-molecular-weight charge transport material (CTM) dissolved therein. The addition of such a low-molecular-weight charge transport material (CTM) to the binder resin lowers the intrinsic mechanical strength of the binder resin, so that the CTL film is fragile and has a low tensile strength. Such lowering of the mechanical strength of the CTL causes the wearing of the photoconductor or forms scratches and cracks in the surface of the photoconductor.

Although some vinyl polymers such as polyvinyl anthracene, polyvinyl pyrene and poly-N-vinylcarbazole have been studied as high-molecular-weight photoconductive materials for forming a charge transport complex for use in the conventional organic photoconductor, such polymers are not satisfactory from the viewpoint of photosensitivity.

In addition, high-molecular-weight materials having charge transporting properties have been also studied to eliminate the shortcomings of the above-mentioned layered photoconductor. For instance, there are proposed an acrylic resin having a triphenylamine structure as reported by M. Stolka et al., in "J. Polym. Sci., vol 21, 969 (1983)"; a vinyl polymer having a hydra zone structure as described in "Japan Hard Copy '89 p. 67"; and polycarbonate resins having a triarylamine structure as disclosed in U.S. Pat. Nos. 4,801,517, 4,806,443, 4,806,444, 4,937,165, 4,959,288, 5,030,532, 5,034,296, and 5,080,989, and Japanese Laid-Open Patent Applications Nos. 64-9964, 3-221522, 2-304456, 4-11627, 4-175337, 4-18371, 4-31404, and 4-133065. However, any materials have not yet been put to practical use.

According to the report of "Physical Review B46 6705 (1992)" by M. A. Abkowitz et al., it is confirmed that the drift mobility of a high-molecular weight charge transport material is lower than that of a low-molecular weight material by one figure. This report is based on the comparison between the photoconductor comprising a low-molecular weight tetraarylbenzidine derivative dispersed in the photoconductive layer and the one comprising a high-molecular polycarbonate having a tetraarylbenzidine structure in its molecule. The reason for this has not been clarified, but it is suggested that the photoconductor employing the high-molecular weight charge transport material produces poor results in terms of the photosensitivity and the residual potential although the mechanical strength of the photoconductor is improved.

Conventionally known representative aromatic polycarbonate resins are obtained by allowing 2,2-bis(4-hydroxyphenyl)propane (hereinafter referred to as bisphenol A) to react with a carbonate precursor material such as phosgene or diphenylcarbonate. Such polycarbonate resins made from bisphenol A are used in many fields because of their excellent characteristics, such as high transparency, high heat resistance, high dimensional accuracy, and high mechanical strength.

For example, this kind of polycarbonate resin is intensively studied as a binder resin for use in an organic photoconductor in the field of electrophotography. A variety of aromatic polycarbonate resins have been proposed as the binder resins for use in the charge transport layer of the layered photoconductor.

As previously mentioned, however, the mechanical strength of the aforementioned aromatic polycarbonate resin is decreased by the addition of the low-molecular-weight charge transport material in the charge transport layer of the layered electrophotographic photoconductor.

**SUMMARY OF THE INVENTION**

It is therefore a first object of the present invention to provide an electrophotographic photoconductor free from the conventional shortcomings, which can show high photosensitivity and high durability.

A second object of the present invention is to provide an aromatic polycarbonate resin that is remarkably useful as a high-molecular-weight charge transport material for use in an organic electrophotographic photoconductor.

The above-mentioned first object of the present invention can be achieved by an electrophotographic photoconductor comprising an electroconductive support, and a photoconductive layer formed thereon comprising as an effective component an aromatic polycarbonate resin having a repeat unit of formula (I):



wherein n is an integer of 5 to 5000; Ar<sup>3</sup> and Ar<sup>4</sup> may be the same or different, and represent a bivalent aromatic hydrocarbon group which may have a substituent or a bivalent heterocyclic group which may have a substituent; Ar<sup>1</sup>, Ar<sup>2</sup>, Ar<sup>5</sup> and Ar<sup>6</sup> each may be the same or different, and represent an aromatic hydrocarbon group which may have a substituent, or a heterocyclic group which may have a substituent; and X is a bivalent aliphatic group, a bivalent cyclic aliphatic group, or



in which R<sup>1</sup> and R<sup>2</sup> are each independently an alkyl group which may have a substituent, an aromatic hydrocarbon group which may have a substituent, or a halogen atom; l and m are each independently an integer of 0 to 4; and p is

an integer of 0 or 1, and when  $p=1$ , Y is a straight-chain, branched or cyclic alkylene group having 1 to 12 carbon atoms,



in which Z is a bivalent aliphatic hydrocarbon group; a is an integer of 0 to 20; b is an integer of 1 to 2000; and R<sup>3</sup> and R<sup>4</sup> are each independently an alkyl group which may have a substituent or an aromatic hydrocarbon group which may have a substituent.

In the above-mentioned electrophotographic photoconductor, both of  $\text{Ar}^3$  and  $\text{Ar}^4$  may be phenylene group in the repeat unit of formula (I) for use in the aromatic polycarbonate resin.

The first object of the present invention can also be achieved by an electrophotographic photoconductor comprising an electroconductive support, and a photoconductive layer formed thereon comprising as an effective component an aromatic polycarbonate resin having a repeat unit of formula (II) and a repeat unit of formula (III), with the composition ratio of the repeat unit of formula (II) to the repeat unit of formula (III) being in the relationship of  $0 < k/(k+j) \leq 1$ :



wherein k is an integer of 5 to 5000; j is an integer of 0 to 5000;  $Ar^3$  and  $Ar^4$  may be the same or different, and represent a bivalent aromatic hydrocarbon group which may have a substituent or a bivalent heterocyclic group which may have a substituent;  $Ar^1$ ,  $Ar^2$ ,  $Ar^3$  and  $Ar^4$  each may be the same or different, and represent an aromatic hydrocarbon group which may have a substituent, or a heterocyclic group

which may have a substituent; and X is a bivalent aliphatic group, a bivalent cyclic aliphatic group, or



10 in which  $R^1$  and  $R^2$  are each independently an alkyl group which may have a substituent, an aromatic hydrocarbon group which may have a substituent, or a halogen atom; 1 and  $m$  are each independently an integer of 0 to 4; and  $p$  is an integer of 0 or 1, and when  $p=1$ ,  $Y$  is a straight-chain, 15 branched or cyclic alkylene group having 1 to 12 carbon atoms.



in which Z is a bivalent aliphatic hydrocarbon group; a is an integer of 0 to 20; b is an integer of 1 to 2000; and R<sup>3</sup> and R<sup>4</sup> are each independently an alkyl group which may have a substituent or an aromatic hydrocarbon group which may have a substituent.



55 The second object of the present invention can be achieved by an aromatic polycarbonate resin having a repeat unit of formula (I):



wherein n is an integer of 5 to 5000; Ar<sup>3</sup> and Ar<sup>4</sup> may be the same or different, and represent a bivalent aromatic hydrocarbon group which may have a substituent or a bivalent heterocyclic group which may have a substituent; Ar<sup>1</sup>, Ar<sup>2</sup>, Ar<sup>5</sup> and Ar<sup>6</sup> each may be the same or different, and represent an aromatic hydrocarbon group which may have a substituent, or a heterocyclic group which may have a substituent; and X is a bivalent aliphatic group, a bivalent cyclic aliphatic group, or



in which R<sup>1</sup> and R<sup>2</sup> are each independently an alkyl group which may have a substituent, an aromatic hydrocarbon group which may have a substituent, or a halogen atom; l and m are each independently an integer of 0 to 4; and p is an integer of 0 or 1, and when p=1, Y is a straight-chain, branched or cyclic alkylene group having 1 to 12 carbon atoms,



in which Z is a bivalent aliphatic hydrocarbon group; a is an integer of 0 to 20; b is an integer of 1 to 2000; and R<sup>3</sup> and R<sup>4</sup> are each independently an alkyl group which may have a substituent or an aromatic hydrocarbon group which may have a substituent.

In the above-mentioned aromatic polycarbonate resin, both of Ar<sup>3</sup> and Ar<sup>4</sup> may be phenylene group in the repeat unit of formula (I).

The second object of the present invention can also be achieved by an aromatic polycarbonate resin having a repeat unit of formula (II) and a repeat unit of formula (III), with the composition ratio of the repeat unit of formula (II) to the repeat unit of formula (III) being in the relationship of 0<k/(k+j)≤1:



wherein k is an integer of 5 to 5000; j is an integer of 0 to 5000; Ar<sup>3</sup> and Ar<sup>4</sup> may be the same or different, and represent a bivalent aromatic hydrocarbon group which may have a substituent or a bivalent heterocyclic group which may have a substituent; Ar<sup>1</sup>, Ar<sup>2</sup>, Ar<sup>5</sup> and Ar<sup>6</sup> each may be the same or different, and represent an aromatic hydrocarbon group which may have a substituent, or a heterocyclic group which may have a substituent; and X is a bivalent aliphatic group, a bivalent cyclic aliphatic group, or



in which R<sup>1</sup> and R<sup>2</sup> are each independently an alkyl group which may have a substituent, an aromatic hydrocarbon group which may have a substituent, or a halogen atom; l and m are each independently an integer of 0 to 4; and p is an integer of 0 or 1, and when p=1, Y is a straight-chain, branched or cyclic alkylene group having 1 to 12 carbon atoms,



in which Z is a bivalent aliphatic hydrocarbon group; a is an integer of 0 to 20; b is an integer of 1 to 2000; and R<sup>3</sup> and R<sup>4</sup> are each independently an alkyl group which may have a substituent or an aromatic hydrocarbon group which may have a substituent.

In the above-mentioned aromatic polycarbonate resin, both of Ar<sup>3</sup> and Ar<sup>4</sup> may be phenylene group in the repeat unit of formula (II).

#### BRIEF DESCRIPTION OF THE DRAWINGS

A more complete appreciation of the invention and many of the attendant advantages thereof will be readily obtained as the same becomes better understood by reference to the following detailed description when considered in connection with the accompanying drawings, wherein:

FIG. 1 is a schematic cross-sectional view of a first example of an electrophotographic photoconductor according to the present invention.

FIG. 2 is a schematic cross-sectional view of a second example of an electrophotographic photoconductor according to the present invention.

FIG. 3 is a schematic cross-sectional view of a third example of an electrophotographic photoconductor according to the present invention.

FIG. 4 is a schematic cross-sectional view of a fourth example of an electrophotographic photoconductor according to the present invention.

FIG. 5 is a schematic cross-sectional view of a fifth example of an electrophotographic photoconductor according to the present invention.

FIG. 6 is a schematic cross-sectional view of a sixth example of an electrophotographic photoconductor according to the present invention.

FIGS. 7 to 9 are IR spectra of aromatic polycarbonate resins Nos. 1, 2 and 3, respectively synthesized in Examples

## DESCRIPTION OF THE PREFERRED EMBODIMENTS

The electrophotographic photoconductor according to the present invention comprises a photoconductive layer comprising (i) an aromatic polycarbonate resin having a repeat unit with a tertiary amino structure, represented by formula (I), or (ii) an aromatic polycarbonate resin having a repeat unit with a tertiary amine structure, represented by formula (II), and a repeat unit of formula (III). Those aromatic polycarbonate resins, which are novel compounds, have charge transporting properties and high mechanical strength, so that the photoconductor of the present invention can exhibit high photosensitivity and excellent durability.

Further, it is preferable that both of  $\text{Ar}^3$  and  $\text{Ar}^4$  be phenylene group in the repeat unit of formula (I), as represented by the following formula (IV):



1-1, 1-2 and 1-3 according to the present invention, taken by use of KBr tablet.

FIGS. 10 to 12 are IR spectra of aromatic polycarbonate resins No. 3', No. 4 and No. 5, respectively synthesized in

wherein n,  $\text{Ar}^1$ ,  $\text{Ar}^2$ ,  $\text{Ar}^5$ ,  $\text{Ar}^6$ , and X are the same as those previously defined in formula (I).

In addition, it is preferable that both of  $\text{Ar}^3$  and  $\text{Ar}^4$  be phenylene group in the repeat unit of formula (II), as represented by the following formula (V):



Examples 1-4, 1-5 and 1-9 according to the present invention, taken by use of an NaCl film.

FIG. 13 is an IR spectrum of a distyrylbenzene compound for the preparation of a dihydroxyl-group-containing diamine compound No. 1 obtained in Preparation Example 1, taken by use of a KBr tablet.

FIG. 14 is an IR spectrum of a dihydroxyl-group-containing diamine compound No. 1 obtained in Preparation Example 1, taken by use of a KBr tablet.

wherein k,  $\text{Ar}^1$ ,  $\text{Ar}^2$ ,  $\text{Ar}^5$ , and  $\text{Ar}^6$  are the same as those previously defined in formula (II).

Those aromatic polycarbonate resins according to the present invention can be obtained by the method of synthesizing a conventional poly carbonate resin, that is, polymerization of a bisphenol and a carbonic acid derivative.

To be more specific, the aromatic polycarbonate resin comprising the repeat unit of formula (II) or (V) with a tertiary amino group can be produced by the ester interchange between a diol compound having a tertiary amino group represented by the following formula (VI) or (VII)

and a bisarylcarbonate compound, or by the polymerization of the diol compound of formula (VI) or (VII) with phosgene in accordance with solution polymerization or interfacial polymerization:



wherein Ar<sup>1</sup> to Ar<sup>6</sup>, and X are the same as those previously defined in formula (I).

When a diol compound of the following formula (VIII) is employed in combination with the diol compound of formula (VI) or (VII) in the course of the polymerization with the phosgene, there can be obtained the aromatic polycarbonate resin of the present invention comprising the repeat unit of formula (II) having a tertiary amino group and the repeat unit of formula (III), or the aromatic polycarbonate resin of the present invention comprising the repeat unit of formula (V) having a tertiary amino group and the repeat unit of formula (III):



wherein X is the same as that previously defined in formula (III).

By such a synthesis method, the aromatic polycarbonate resin provided with the desired characteristics can be obtained. Further, the composition ratio of the repeat unit of formula (II) to the repeat unit of formula (III), or that of the repeat unit of formula (V) to the repeat unit of formula (III) can be selected within a wide range in light of the desired characteristics of the obtained aromatic polycarbonate resin.

The aromatic polycarbonate resin of the present invention comprising the repeat unit having a tertiary amino group, represented by formula (I) or (IV), can be obtained by polymerizing the diol compound having a tertiary amino group represented by formula (VI) or (VII) with a bischloroformate compound derived from the diol compound of formula (VIII) in accordance with solution polymerization or interfacial polymerization. Alternatively, the above-mentioned aromatic polycarbonate resin can also be obtained by polymerizing a bischloroformate derived from the diol compound of formula (VI) or (VII) with the diol compound of formula (VIII).

According to the ester interchange method, a diol compound and a bisarylcarbonate compound are mixed in the presence of an inert gas, and the polymerization reaction is

generally carried out at temperature in the range of 120° to 350° C. under reduced pressure. The pressure in the reaction system is stepwise reduced to 1 mmHg or less in order to distill away the phenols generated during the reaction from

the reaction system. The reaction is commonly terminated in about one to 4 hours. When necessary, a molecular weight modifier and an antioxidant may be added to the reaction system. As the bisarylcarbonate compound, diphenyl carbonate, di-p-tolyl carbonate, phenyl-p-tolyl carbonate, di-p-chlorophenyl carbonate and dinaphthyl carbonate can be employed.

The polymerization of a diol compound with the phosgene is commonly carried out in the presence of an agent for deacidifying and a solvent. In this case, hydroxides of alkali metals such as sodium hydroxide and potassium hydroxide, and pyridine can be used as the deacidifying agents in the above reaction. As the solvent, halogenated hydrocarbon solvents such as dichloromethane and chlorobenzene can be employed. In addition, a catalyst such as tertiary amine or a quaternary ammonium salt may be used to accelerate the reaction speed. Furthermore, it is also desirable to use phenol or p-tert-butylphenol as a molecular weight modifier. The polymerization reaction is generally carried out at temperature in the range of 0° to 40° C. In this case, the polymerization is terminated in several minutes to 5 hours. It is desirable to maintain the reaction system to pH 10 or more.

In the case of the polymerization of a diol compound with a bischloroformate compound, the diol is dissolved in a proper solvent to prepare a solution of the diol compound, and a deacidifying agent and the bischloroformate compound are added to the above prepared diol solution. In this case, tertiary amine compounds such as trimethylamine, triethylamine and tripropylamine, and pyridine can be used as the deacidifying agents. Examples of the solvent for use in the above-mentioned polymerization reaction are halogenated hydrocarbon solvents such as dichloromethane, dichloroethane, trichloroethane, tetrachloroethane, trichloroethylene, and chloroform; and cyclic ethers such as tetrahydrofuran and dioxane. In addition, it is desirable to use phenol or p-tert-butylphenol as a molecular weight modifier. The reaction temperature is generally in the range

of 0 to 40° C. In this case, the polymerization is generally terminated in several minutes to 5 hours.

To the aromatic polycarbonate resin produced by the previously mentioned methods, various additives such as an antioxidant, a light stabilizer, a thermal stabilizer, a lubricant and a plasticizer can be added when necessary.

As previously mentioned, the aromatic polycarbonate resin according to the present invention is a homopolymer comprising a repeat unit of (II) or (V), an alternating copolymer comprising the repeat unit of formula (I) or (IV), or a random copolymer or block copolymer comprising the repeat unit of (II) or (V) and the repeat unit of (III).

It is preferable that the aromatic polycarbonate resin according to the present invention thus obtained have a number-average molecular weight of 1,000 to 1,000,000, more preferably in the range of 5,000 to 500,000 when expressed by the styrene-reduced value.

The above-mentioned diol compound having a tertiary amine group, represented by the formula (VI) or (VII), which is an intermediate for preparation of the aromatic polycarbonate resin according to the present invention, will now be explained in detail.

In the present invention, there can be employed a dihydroxyl-group-containing diamine compound represented by the following formula (IX), which is a novel compound, as the diol compound having a tertiary amine group:



wherein R<sup>11</sup> to R<sup>16</sup>, which may be the same or different, are each independently an alkyl group which may have a substituent, a halogen atom, an aromatic hydrocarbon group which may have a substituent, or a heterocyclic group which may have a substituent; a and b are each independently an integer of 0 to 5; and c, d, e and f are each independently an integer of 0 to 4.

Namely, such a dihydroxyl-group-containing diamine compound can be used as an intermediate for preparation of the aromatic polycarbonate resin according to the present invention.

In the formula (IX), the alkyl group represented by R<sup>11</sup> to R<sup>16</sup> is a straight-chain or branched alkyl group having 1 to 5 carbon atoms. The above alkyl group may have a substituent such as a fluorine atom, cyano group, or a phenyl group which may have a substituent selected from the group consisting of a halogen atom and an alkyl group having 1 to 5 carbon atoms.

Specific examples of the above alkyl group include methyl group, ethyl group, n-propyl group, i-propyl group, tert-butyl group, sec-butyl group, n-butyl group, i-butyl group, trifluoromethyl group, 2-cyanoethyl group, benzyl group, 4-chlorobenzyl group, and 4-methylbenzyl group.

Examples of the aromatic hydrocarbon group represented by R<sup>11</sup> to R<sup>16</sup> are phenyl group, biphenyl group, terphenyl group, naphthyl group, anthryl group, pyrenyl group, fluorenyl group, 9,9-dimethyl-2-fluorenyl group, azulenyl group, triphenylenyl group, chrysene group, and a group of the following formula (X);



wherein R<sup>17</sup> is a hydrogen atom, an alkyl group which may have a substituent, an alkoxy group, a halogen atom, an aromatic hydrocarbon group which may have a substituent, nitro group, cyano group or a substituted amino group; and W is selected from the group consisting of —O—, —S—, —SO—, —SO<sub>2</sub>—, —CO— and the following bivalent groups:



in which R<sup>18</sup> is a hydrogen atom, an alkyl group which may have a substituent, or an aromatic hydrocarbon group which may have a substituent; and r and s are each independently an integer of 1 to 12.

In the case where R<sup>17</sup> and R<sup>18</sup> represent an aromatic hydrocarbon group which may have a substituent, the same aromatic hydrocarbon groups as mentioned above are usable.

In the case where R<sup>17</sup> and R<sup>18</sup> represent an alkyl group which may have a substituent, there can be employed the same alkyl groups as mentioned in the definition of the alkyl group represented by R<sup>11</sup> to R<sup>16</sup>.

In the case where R<sup>17</sup> represents a substituted amino group, there can be employed a group of:



in which R<sup>19</sup> and R<sup>20</sup> are each independently an alkyl group which may have a substituent, or an aromatic hydrocarbon group which may have a substituent or a heterocyclic group. In addition, R<sup>19</sup> and R<sup>20</sup> may form a ring in combination with each other, or in combination with a carbon atom of the aryl group, thereby forming piperidino group, morpholino group and julolidyl group.

When R<sup>11</sup> to R<sup>17</sup> represent a halogen atom, there can be employed a fluorine atom, chlorine atom, bromine atom, and iodine atom.

**13**

The dihydroxyl-group-containing diamine compound of formula (IX) can be synthesized by the conventional method in accordance with the reaction schemes shown below.

A corresponding aldehyde compound having an alkoxy group, represented by formula (XI), is allowed to react with a corresponding bis(phosphonate) compound of formula

**14**

(XII) by the modified Wittig reaction, so that a distyrylbenzene compound of formula (XIII) can be obtained.

Furthermore, cleavage of an ether linkage of the alkoxy group is carried out in the distyrylbenzene compound of formula (XIII), so that a dihydroxyl-group-containing diamine compound of formula (IX) can be obtained.





wherein R<sup>11</sup> to R<sup>16</sup>, and a to f are the same as those previously defined in formula (IX); and R<sup>21</sup> and R<sup>22</sup> are each independently a lower alkyl group.

In the above-mentioned modified Wittig reaction, potassium-t-butoxide, sodium hydroxide, potassium hydroxide, sodium amido, sodium methylate, and potassium methylate are preferably used as the basic catalysts.

Examples of the reaction solvent used in the above-mentioned condensation reaction are methanol, ethanol, isopropanol, butanol, 2-methoxyethanol, 1,2-dimethoxyethane, bis(2-methoxyethyl)ether, dioxane, tetrahydrofuran, toluene, xylene, dimethyl sulfoxide, N,N-dimethylformamide, N-methylpyrrolidone and 1,3-dimethyl-2-imidazolidinone. Of these solvents, a polar solvent such as N,N-dimethylformamide or dimethyl sulfoxide is preferably employed.

The reaction temperature in the modified Wittig reaction may be determined within a wide range depending on (1) the stability of the employed solvent with respect to the employed basic catalyst, (2) the reactivity of the condensed components, and (3) the reactivity of the employed basic catalyst as a condensation agent in the solvent. For instance, when a polar solvent is employed, the reaction temperature is in the range of room temperature to 100° C., preferably in the range of room temperature to 80° C. The reaction temperature may be further increased when it is desired to curtail the reaction time, or the activity of a condensation agent to be employed is low.

The cleavage of the ether linkage of the alkoxyl group in the distyrylbenzene compound of formula (XIII) can be carried out using sodium thioethoxide or trimethylsilyl iodide.

When the above-mentioned sodium thioethoxide is employed for the cleavage of the other linkage, a solvent such as N,N-dimethylformamide or triamide of hexamethyl phosphoric acid is preferably employed. In such a case, the reaction temperature is in the range of room temperature to 180° C., preferably in the range of 10 to 150° C. The reaction time varies with the reactivity of the alkoxyl group, so that

the reaction may be terminated in about 20 minutes or it may take 10 hours or more. The cleavage of the ether linkage can be carried out similarly by using sodium thiomethoxide instead of sodium thioethoxide.

When trimethylsilyl iodide is employed for the cleavage of the ether linkage, a solvent such as dichloromethane, chloroform, carbon tetrachloride, sulfolane or acetonitrile is preferably employed. In this case, the reaction temperature is in the range of room temperature to 100° C. In stead of trimethylsilyl iodide, trimethylsilyl chloride and sodium iodide may be employed.

Furthermore, the cleavage of the ether linkage can also be carried out using a reagent such as hydriodic acid.

The bis(phosphonate) compound of formula (XII) can be readily produced by allowing a corresponding halogen compound to react with trialkyl phosphite under the application of heat thereto without any solvent, or in an organic solvent such as toluene, xylene or N,N-dimethylformamide.

A variety of materials such as a polycarbonate resin, polyester resin, polyurethane resin and epoxy resin can be obtained by deriving from the hydroxyl group of the above-mentioned dihydroxyl-group-containing diamine compound. In other words, the dihydroxyl-group-containing diamine compound of formula (IX) for use in the present invention is considered to be useful as an intermediate for the preparation of the above-mentioned materials. In particular, an organic polymer such as a polycarbonate resin prepared from the above-mentioned dihydroxyl-group-containing diamine compound is useful as the organic photoconductive material.

The polycarbonate resin according to the present invention will now be explained in detail.

In the repeat units of the aromatic polycarbonate resins, represented by formulae (I), (II), (IV) and (V), and the diol compounds represented by formulae (VI) and (VII), Ar<sup>1</sup>, Ar<sup>2</sup>, Ar<sup>5</sup> and Ar<sup>6</sup> represent an aromatic hydrocarbon group or a heterocyclic group, as previously mentioned.

Examples of the aromatic hydrocarbon group represented by Ar<sup>1</sup>, Ar<sup>2</sup>, Ar<sup>5</sup> and Ar<sup>6</sup> are phenyl group, naphthyl group,

biphenyl group, terphenyl group, pyrenyl group, fluorenyl group, and 9,9-dimethyl-2-fluorenyl group.

Examples of the heterocyclic group represented by  $\text{Ar}^1$ ,  $\text{Ar}^2$ ,  $\text{Ar}^5$  and  $\text{Ar}^6$  are thiienyl group, benzothienyl group, furyl group, benzofuranyl group and carbazolyl group.

The above-mentioned aromatic hydrocarbon group and heterocyclic group represented by  $\text{Ar}^1$ ,  $\text{Ar}^2$ ,  $\text{Ar}^5$  and  $\text{Ar}^6$  may have a substituent.

Examples of such a substituent for  $\text{Ar}^1$ ,  $\text{Ar}^2$ ,  $\text{Ar}^5$  and  $\text{Ar}^6$  are as follows:

(1) A halogen atom, cyano group, and nitro group.

(2) An alkyl group, preferably a straight chain or branched alkyl group having 1 to 12 carbon atoms, more preferably having 1 to 8 carbon atoms, further preferably having 1 to 4 carbon atoms. The alkyl group may have a substituent such as a fluorine atom, hydroxyl group, cyano group, an alkoxy group having 1 to 4 carbon atoms, or a phenyl group which may have a substituent selected from the group consisting of a halogen atom, an alkyl group having 1 to 4 carbon atoms, and an alkoxy group having 1 to 4 carbon atoms.

Specific examples of such an alkyl group are methyl group, ethyl group, n-propyl group, i-propyl group, t-butyl group, s-butyl group, n-butyl group, i-butyl group, trifluoromethyl group, 2-hydroxyethyl group, 2-cyanoethyl group, 2-ethoxyethyl group, 2-methoxyethyl group, benzyl group, 4-chlorobenzyl group, 4-methylbenzyl group, and 4-methoxybenzyl group.

(3) An alkoxy group ( $-\text{OR}^5$ ) in which  $\text{R}^5$  is the same alkyl group as previously defined in (2).

Specific examples of such an alkoxy group are methoxy group, ethoxy group, n-propoxy group, i-propoxy group, t-butoxy group, n-butoxy group, s-butoxy group, i-butoxy group, 2-hydroxyethoxy group, 2-cyanoethoxy group, benzylxy group, 4-methylbenzylxy group, and trifluoromethoxy group.

(4) An aryloxy group. Examples of the aryl group for use in the aryloxy group are phenyl group and naphthyl group. The aryloxy group may have a substituent such as an alkoxy group having 1 to 4 carbon atoms, an alkyl group having 1 to 4 carbon atoms, or a halogen atom.

Specific examples of the aryloxy group are phenoxy group, 1-naphthoxy group, 2-naphthoxy group, 4-methylphenoxy group, 4-methoxyphenoxy group, 4-chlorophenoxy group, and 6-methyl-2-naphthoxy group.

(5) A substituted mercapto group or an arylmercapto group. Specific examples of the substituted mercapto group and arylmercapto group include methylthio group, ethylthio group, phenylthio group, and p-methylphenylthio group.

(6) An alkyl-substituted amino group. The same alkyl group as defined in (2) can be used for the alkyl-substituted amino group.

Specific examples of the alkyl-substituted amino group are dimethylamino group, diethylamino group, N-methyl-N-propylamino group, and N,N-dibenzylamino group.

(7) An acyl group such as acetyl group, propionyl group, butyryl group, malonyl group, or benzoyl group.

The bivalent aromatic hydrocarbon group represented by  $\text{Ar}^3$  and  $\text{Ar}^4$  is a bivalent group derived from one aromatic hydrocarbon group selected from the group consisting of benzene, naphthalene, biphenyl terphenyl, pyrene, fluorene, and 9,9-dimethylfluorene.

The bivalent heterocyclic group represented by  $\text{Ar}^3$  and  $\text{Ar}^4$  is a bivalent group derived from one heterocyclic group selected from the group consisting of thiophene, benzothiophene, furan, benzofuran and carbazole. Further, for the bivalent heterocyclic group represented by  $\text{Ar}^3$  and

$\text{Ar}^4$ , there can be employed diphenyl ether group in which two aryl groups are bonded via oxygen, or diphenyl thioether group in which two aryl groups are bonded via sulfur.

Such a bivalent aromatic hydrocarbon group and a bivalent heterocyclic group represented by  $\text{Ar}^3$  and  $\text{Ar}^4$  may also have the same substituent as mentioned above, that is, a halogen atom, cyano group, nitro group, an alkyl group having 1 to 12 carbon atoms, an alkoxy group having 1 to 12 carbon atoms, an aryloxy group, a substituted mercapto group, an arylmercapto group, an alkyl-substituted amino group, or an acyl group.

When  $\text{R}^1$  to  $\text{R}^4$  in formula (I) or (II) represent an alkyl group which may have a substituent, the same alkyl groups as previously mentioned in the definition (2) of alkyl group can be employed. When  $\text{R}^1$  to  $\text{R}^4$  represent an aromatic hydrocarbon group which may have a substituent, there can be employed a substituted or unsubstituted phenyl group, or a substituted or unsubstituted biphenyl group.

Examples of the diol compound represented by formula (VIII) include aliphatic diols such as 1,3-propanediol, 1,4-butane diol, 1,5-pentanediol, 1,6-hexanediol, 1,8-octanediol, 1,10-decanediol, 2-methyl-1,3-propanediol, 2,2-dimethyl-1,3-propanediol, 2-ethyl-1,3-propanediol, diethylene glycol, triethylene glycol, polyethylene glycol and polytetramethylene ether glycol; and cyclic aliphatic diols such as 1,4-cyclohexanediol, 1,3-cyclohexanediol and cyclohexane-1,4-dimethanol.

Examples of the diol having an aromatic ring are as follows: 4,4'-dihydroxydiphenyl, bis(4-hydroxyphenyl) methane, 1,1-bis(4-hydroxyphenyl)ethane, 1,1-bis(4-hydroxyphenyl)-1-phenylethane, 2,2-bis(4-hydroxyphenyl) propane, 2,2-bis(3-methyl-4-hydroxyphenyl)propane, 1,1-bis(4-hydroxyphenyl)cyclohexane, 1,1-bis(4-hydroxyphenyl)cyclopentane, 2,2-bis(3-phenyl-4-hydroxyphenyl)propane, 2,2-bis(3-isopropyl-4-hydroxyphenyl)propane, 2,2-bis(4-hydroxyphenyl)butane, 2,2-bis(3,5-dimethyl-4-hydroxyphenyl)propane, 2,2-bis(3,5-dibromo-4-hydroxyphenyl)propane, 4,4'-dihydroxydiphenylsulfone, 4,4'-dihydroxydiphenylsulfoxide, 4,4'-dihydroxydiphenylsulfide, 3,3'-dimethyl-4,4'-dihydroxydiphenylsulfide, 4,4'-dihydroxydiphenyloxide, 2,2-bis(4-hydroxyphenyl)hexafluoropropane, 9,9-bis(4-hydroxyphenyl)fluorene, 9,9-bis(4-hydroxyphenyl)xanthene, ethylene glycol-bis(4-hydroxybenzoate), diethylene glycol-bis(4-hydroxybenzoate), triethylene glycol-bis(4-hydroxybenzoate), 1,3-bis(4-hydroxyphenyl)-tetramethyl disiloxane, and phenol-modified silicone oil.

In the photoconductors according to the present invention, at least one of the previously mentioned aromatic polycarbonate resins is contained in the photoconductive layers 2, 2a, 2b, 2c, 2d, and 2e. The aromatic polycarbonate resin can be employed in different ways, for example, as shown in FIGS. 1 through 6.

In the photoconductor as shown in FIG. 1, a photoconductive layer 2 is formed on an electroconductive support 1, which photoconductive layer 2 comprises an aromatic polycarbonate resin of the present invention and a sensitizing dye, with the addition thereto of a binder agent (binder resin) when necessary. In this photoconductor, the aromatic polycarbonate resin works as a photoconductive material, through which charge carriers which are necessary for the light decay of the photoconductor are generated and transported. However, the aromatic polycarbonate resin itself scarcely absorbs light in the visible light range and, therefore, it is necessary to add a sensitizing dye which absorbs light in the visible light range in order to form latent electrostatic images by use of visible light.

Referring to FIG. 2, there is shown an enlarged cross-sectional view of another embodiment of an electrophotographic photoconductor according to the present invention. In this photoconductor, there is formed a photoconductive layer **2a** on an electroconductive support **1**. The photoconductive layer **2a** comprises a charge transport medium **4** comprising (i) an aromatic polycarbonate resin of the present invention, optionally in combination with a binder agent, and (ii) a charge generation material **3** dispersed in the charge transport medium **4**. In this embodiment, the aromatic polycarbonate resin (or a mixture of the aromatic polycarbonate resin and the binder agent) constitutes the charge transport medium **4**. The charge generation material **3**, which is, for example, an inorganic material or an organic pigment, generates charge carriers. The charge transport medium **4** accepts the charge carriers generated by the charge generation material **3** and transports those charge carriers.

In this electrophotographic photoconductor, it is basically necessary that the light-absorption wavelength regions of the charge generation material **3** and the aromatic polycarbonate resin not overlap in the visible light range. This is because, in order that the charge generation material **3** produce charge carriers efficiently, it is necessary that light pass through the charge transport medium **4** and reach the surface of the charge generation material **3**. Since the aromatic polycarbonate resin comprising the repeat unit of formula (I) do not substantially absorb light in the visible range, it can work effectively as a charge transport material when used with the charge generation material **3** which absorbs the light in the visible region and generates charge carriers. The charge transport medium **4** may further comprise a low-molecular weight charge transport material in combination.

Referring to FIG. 3, there is shown an enlarged cross-sectional view of a further embodiment of an electrophotographic photoconductor according to the present invention. In the figure, there is formed on an electroconductive support **1** a two-layered photoconductive layer **2b** comprising a charge generation layer **5** containing the charge generation material **3**, and a charge transport layer **4** comprising an aromatic polycarbonate resin of the present invention.

In this photoconductor, light which has passed through the charge transport layer **4** reaches the charge generation layer **5**, and charge carriers are generated within the charge generation layer **5**. The charge carriers which are necessary for the light decay for latent electrostatic image formation are generated by the charge generation material **3**, and accepted and transported by the charge transport layer **4**. The generation and transportation of the charge carriers are performed by the same mechanism as that in the photoconductor shown in FIG. 2.

In this case, the charge transport layer **4** comprises the aromatic polycarbonate resin, optionally in combination with a binder agent. Furthermore, in order to increase the efficiency of generating the charge carriers, the charge generation layer **5** may further comprise the aromatic polycarbonate resin of the present invention, and the photoconductive layer **2b** including the charge generation layer **5** and the charge transport layer **4** may further comprise a low-molecular weight charge transport material. This can be applied to the embodiments of FIGS. 4 to 6 to be described later.

In the electrophotographic photoconductor of FIG. 3, a protective layer **6** may be provided on the charge transport layer **4** as shown in FIG. 4. The protective layer **6** may comprise the aromatic polycarbonate resin of the present invention, optionally in combination with a binder agent. In

such a case, it is effective that the protective layer **6** be provided on a charge transport layer in which a low-molecular weight charge transport material is dispersed. The protective layer **6** may be provided on the photoconductive layer **2a** of the photoconductor as shown in FIG. 2.

Referring to FIG. 5, there is shown still another embodiment of an electrophotographic photoconductor according to the present invention. In this figure, the overlaying order of the charge generation layer **5** and the charge transport layer **4** comprising the aromatic polycarbonate resin is reversed in view of the electrophotographic photoconductor as shown in FIG. 3. The mechanism of the generation and transportation of charge carriers is substantially the same as that of the photoconductor shown in FIG. 3.

In the above photoconductor of FIG. 5, a protective layer **6** may be formed on the charge generation layer **5** as shown in FIG. 6 in light of the mechanical strength of the photoconductor.

When the electrophotographic photoconductor according to the present invention as shown in FIG. 1 is prepared, at least one aromatic polycarbonate resin of the present invention is dissolved in a solvent, with the addition thereto of a binder agent when necessary. To the thus prepared solution, a sensitizing dye is added, so that a photoconductive layer **2** coating liquid is prepared. The thus prepared photoconductive layer coating liquid is coated on an electroconductive support **1** and dried, so that a photoconductive layer **2** is formed on the electroconductive support **1**.

It is preferable that the thickness of the photoconductive layer **2** be in the range of 3 to 50  $\mu\text{m}$ , more preferably in the range of 5 to 20  $\mu\text{m}$ . It is preferable that the amount of aromatic polycarbonate resin of the present invention be in the range of 30 to 100 wt. % of the total weight of the photoconductive layer **2**.

It is preferable that the amount of sensitizing dye for use in the photoconductive layer **2** be in the range of 0.1 to 5 wt. %, more preferably in the range of 0.5 to 3 wt. % of the total weight of the photoconductive layer **2**.

Specific examples of the sensitizing dye for use in the present invention are triarylmethane dyes such as Brilliant Green, Victoria Blue B, Methyl Violet, Crystal Violet and Acid Violet 6B; xanthene dyes such as Rhodamine B, Rhodamine 6G, Rhodamine G Extra, Eosin S, Erythrosin, Rose Bengal and Fluoresceine; thiazine dyes such as Methylene Blue; and cyanine dyes such as cyanin.

The electrophotographic photoconductor as shown in FIG. 2 can be obtained by the following method:

The finely-divided particles of the charge generation material **3** are dispersed in a solution in which at least one aromatic polycarbonate resin of the present invention, or a mixture of the aromatic polycarbonate resin and the binder agent is dissolved, so that a coating liquid for the photoconductive layer **2a** is prepared. The coating liquid thus prepared is coated on the electroconductive support **1** and then dried, whereby the photoconductive layer **2a** is provided on the electroconductive support **1**.

It is preferable that the thickness of the photoconductive layer **2a** be in the range of 3 to 50  $\mu\text{m}$ , more preferably in the range of 5 to 20  $\mu\text{m}$ . It is preferable that the amount of aromatic polycarbonate resin for use in the photoconductive layer **2a** be in the range of 40 to 100 wt. % of the total weight of the photoconductive layer **2a**.

It is preferable that the amount of charge generation material **3** for use in the photoconductive layer **2a** be in the range of 0.1 to 50 wt. %, more preferably in the range of 1 to 20 wt. % of the total weight of the photoconductive layer **2a**.

Specific examples of the charge generation material **3** for use in the present invention are as follows: inorganic materials such as selenium, selenium—tellurium, cadmium sulfide, cadmium sulfide—selenium and  $\alpha$ -silicone; and organic pigments such as an azo pigment, for example, C.I. Pigment Blue 25 (C.I. 21180), C.I. Pigment Red 41 (C.I. 21200), C.I. Acid Red 52 (C.I. 45100), C.I. Basic Red 3 (C.I. 45210), an azo pigment having a carbazole skeleton (Japanese Laid-Open Patent Application 53-95033), an azo pigment having a distyryl benzene skeleton (Japanese Laid-Open Patent Application 53-133445), an azo pigment having a triphenylamine skeleton (Japanese Laid-Open Patent Application 53-132347), an azo pigment having a dibenzothiophene skeleton (Japanese Laid-Open Patent Application 54-21728), an azo pigment having an oxadiazole skeleton (Japanese Laid-Open Patent Application 54-12742), an azo pigment having a fluorenone skeleton (Japanese Laid-Open Patent Application 54-22834), an azo pigment having a bisstilbene skeleton (Japanese Laid-Open Patent Application 54-17733), an azo pigment having a distyryl oxadiazole skeleton (Japanese Laid-Open Patent Application 54-2129), and an azo pigment having a distyryl carbazole skeleton (Japanese Laid-Open Patent Application 54-14967); a phthalocyanine pigment such as C.I. Pigment Blue 16 (C.I. 74100); an indigo pigment such as C.I. Vat Brown 5 (C.I. 73410) and C.I. Vat Dye (C.I. 73030); and a perylene pigment such as Algol Scarlet B and Indanthrene Scarlet R (made by Bayer Co., Ltd.). These charge generation materials may be used alone or in combination.

The electrophotographic photoconductor shown in FIG. 3 can be obtained by the following method:

To provide the charge generation layer **5** on the electroconductive support **1**, the charge generation material is vacuum-deposited on the electroconductive support **1**. Alternatively, the finely-divided particles of the charge generation material **3** are dispersed in an appropriate solvent, together with the binder agent when necessary, so that a coating liquid for the charge generation layer **5** is prepared. The thus prepared coating liquid is coated on the electroconductive support **1** and dried, whereby the charge generation layer **5** is formed on the electroconductive support **1**. The charge generation layer **5** may be subjected to surface treatment by buffing and adjustment of the thickness thereof if required. On the thus formed charge generation layer **5**, a coating liquid in which at least one aromatic polycarbonate resin of the present invention, optionally in combination with a binder agent is dissolved is coated and dried, so that the charge transport layer **4** is formed on the charge generation layer **5**. In the charge generation layer **5**, the same charge generation materials as employed in the above-mentioned photoconductive layer **2a** can be used.

The thickness of the charge generation layer **5** is 5  $\mu\text{m}$  or less, preferably 2  $\mu\text{m}$  or less. It is preferable that the thickness of the charge transport layer **4** be in the range of 3 to 50  $\mu\text{m}$ , more preferably in the range of 5 to 20  $\mu\text{m}$ .

When the charge generation layer **5** is provided on the electroconductive support **1** by coating the dispersion in which finely-divided particles of the charge generation material **3** are dispersed in an appropriate solvent, it is preferable that the amount of finely-divided particles of the charge generation material **3** for use in the charge generation

layer **5** be in the range of 10 to 100 wt. %, more preferably in the range of about 50 to 100 wt. % of the total weight of the charge generation layer **5**. It is preferable that the amount of aromatic polycarbonate resin of the present invention for use in the charge transport layer **4** be in the range of 40 to 100 wt. % of the total weight of the charge transport layer **4**.

The photoconductive layer **2b** of the photoconductor shown in FIG. 3 may comprise a low-molecular-weight charge transport material as previously mentioned.

Examples of the low-molecular-weight charge transport material for use in the present invention are as follows: oxazole derivatives, oxadiazole derivatives (Japanese Laid-Open Patent Applications 52-139065 and 52-139066), imidazole derivatives, triphenylamine derivatives (Japanese Laid-Open Patent Application 3-285960), benzidine derivatives (Japanese Patent Publication 58-32372),  $\alpha$ -phenylstilbene derivatives (Japanese Laid-Open Patent Application 57-73075), hydrazone derivatives (Japanese Laid-Open Patent Applications 55-154955, 55-156954, 55-52063, and 56-81850), triphenylmethane derivatives (Japanese Patent Publication 51-10983), anthracene derivatives (Japanese Laid-Open Patent Application 51-94829), styryl derivatives (Japanese Laid-Open Patent Applications 56-29245 and 58-198043), carbazole derivatives (Japanese Laid-Open Patent Application 58-58552), and pyrene derivatives (Japanese Laid-Open Patent Application 2-94812).

To prepare the photoconductor shown in FIG. 4, a coating liquid for the protective layer **6** is prepared by dissolving the aromatic polycarbonate resin of the present invention, optionally in combination with the binder agent, in a solvent, and the thus obtained coating liquid is coated on the charge transport layer **4** of the photoconductor shown in FIG. 3, and dried.

It is preferable that the thickness of the protective layer **6** be in the range of 0.15 to 10  $\mu\text{m}$ . It is preferable that the amount of aromatic polycarbonate resin of the present invention for use in the protective layer **6** be in the range of 40 to 100 wt. % of the total weight of the protective layer **6**.

The electrophotographic photoconductor shown in FIG. 5 can be obtained by the following method:

The aromatic polycarbonate resin of the present invention, optionally in combination with the binder agent, is dissolved in a solvent to prepare a coating liquid for the charge transport layer **4**. The thus prepared coating liquid is coated on the electroconductive support **1** and dried, whereby the charge transport layer **4** is provided on the electroconductive support **1**. On the thus formed charge transport layer **4**, a coating liquid prepared by dispersing the finely-divided particles of the charge generation material **3** in a solvent in which the binder agent may be dissolved when necessary, is coated by spray coating and dried, so that the charge generation layer **5** is provided on the charge transport layer **4**. The amount ratios of the components contained in the charge generation layer **5** and charge transport layer **4** are the same as those previously described in FIG. 3.

The electrophotographic photoconductor shown in FIG. 6 can be fabricated by forming a protective layer **6** on the charge generation layer **5** of the photoconductor shown in FIG. 5.

To obtain any of the aforementioned photoconductor u of the present invention, a metallic plate or foil made of aluminum, a plastic film on which a metal such as aluminum is deposited, and a sheet of paper which has been treated so as to be electroconductive can be employed as the electroconductive support 1.

Specific examples of the binder agent used in the preparation of the photoconductor according to the present invention are condensation resins such as polyamide, polyurethane, polyester, epoxy resin, polyketone and polycarbonate; and vinyl polymers such as polyvinylketone, polystyrene, poly-N-vinylcarbazole and polyacrylamide. All the resins having insulating properties and adhesion properties can be employed.

Some plasticizers may be added to the above-mentioned binder agents, when necessary. Examples of the plasticizer for use in the present invention are halogenated paraffin, dimethylnaphthalene and dibutyl phthalate. Further, a variety of additives such as an antioxidant, a light stabilizer, a thermal stabilizer and a lubricant may also be contained in the binder agents when necessary.

Furthermore, in the electrophotographic photoconductor according to the present invention, an intermediate layer such as an adhesive layer or a barrier layer may be interposed between the electroconductive support and the photoconductive layer when necessary. Examples of the material for use in the intermediate layer are polyamide, nitrocellulose and aluminum oxide. It is preferable that the thickness of the intermediate layer be 1  $\mu\text{m}$  or less.

When copying is performed by use of the photoconductor according to the present invention, the surface of the photoconductor is uniformly charged to a predetermined polarity in the dark. The uniformly charged photoconductor is exposed to a light image so that a latent electrostatic image is formed on the surface of the photoconductor. The thus formed latent electrostatic image is developed to a visible image by a developer, and the developed image can be transferred to a sheet of paper when necessary.

The photosensitivity and the durability of the electrophotographic photoconductor according to the present invention are remarkably improved.

Other features of this invention will become apparent in the course of the following description of exemplary embodiments, which are given for illustration of the invention and are not intended to be limiting thereof.

#### PREPARATION EXAMPLE 1

[Preparation of dihydroxyl-group-containing diamine compound No. 1, i.e. N',N',N'',N''-tetra(4-methylphenyl)-1,4-bis [ $\alpha$ -(4-hydroxyphenyl)styryl] benzene-4',4"-diamine]

28.93 g (0.096 mol) of 4-formyl-4',4"-dimethyltriphenylamine represented by the following formula (1) and 23.62 g (0.04 mol) of a bis(phosphonate)

compound represented by the following formula (2) were dissolved in 300 ml of DMF, and the thus obtained solution was cooled to 15° C.



40 To the above prepared solution, 13.47 g (0.12 mol) of potassium tert-butoxide (t-BuOK) was dropwise added over a period of 30 minutes, with the temperature of the mixture being maintained at 15° to 25° C.

45

50 After stirring for 2.0 hours, the reaction mixture was poured into 3,000 ml of water. After the resulting precipitate was separated from the mixture by filtration, it was washed with water and dried under reduced pressure. The thus obtained crude product was chromatographed on a silica gel column using as a developing solvent a mixed solvent of toluene and cyclohexane at a mixing ratio of 1:1, whereby 24.92 g of a distyrylbenzene compound represented by formula (3) was obtained in a yield of 70.40%. The above-mentioned distyrylbenzene compound was amorphous.



(3)

20

The results of the elemental analysis of the above-mentioned distyrylbenzene compound are as follows:

| Elemental analysis: |       |      |
|---------------------|-------|------|
| % C                 | % H   | % N  |
| Found               | 86.90 | 6.40 |
|                     |       | 3.06 |

chromatographed on a silica gel column using as a developing solvent a mixed solvent of toluene and ethyl acetate at a mixing ratio of 20:3, whereby 18.76 g of a dihydroxyl-group-containing diamine compound No. 1 represented by formula (4), that is, N',N',N'',N''-tetra(4-methylphenyl)-1,4-bis[ $\alpha$ -(4-hydroxyphenyl)styryl]benzene-4',4"-diamine was obtained in a yield of 86.21%. The above-mentioned dihydroxyl-group-containing diamine compound was amorphous.

[Dihydroxyl-group-containing diamine compound No. 1]



45

-continued

| Elemental analysis: |       |      |
|---------------------|-------|------|
| % C                 | % H   | % N  |
| Calcd.              | 86.84 | 6.38 |
|                     |       | 3.16 |

An infrared spectrum of this distyrylbenzene compound, taken by use of a KBr tablet, is shown in FIG. 13.

23.01 g (0.026 mol) of the distyrylbenzene compound represented by formula (3) and 20.0 g (0.24 mol) of sodium thioethoxide were dissolved in 300 ml of dry DMF. Then, the mixture was refluxed for 5 hours with stirring under the application of heat thereto, and then the reaction was terminated.

Thereafter, the reaction mixture was cooled to room temperature, and 20 ml of concentrated hydrochloric acid was added to the reaction mixture. The resultant solution was washed with water and dried over anhydrous magnesium sulfate, and then a solvent was distilled away from the reaction mixture. The thus obtained crude product was

50 The results of the elemental analysis of the dihydroxyl-group-containing diamine compound No. 1 are as follows:

| Elemental analysis: |       |      |
|---------------------|-------|------|
| % C                 | % H   | % N  |
| Found               | 86.85 | 6.14 |
| Calcd.              | 86.88 | 6.12 |
|                     |       | 3.19 |
|                     |       | 3.27 |

55 An infrared spectrum of this dihydroxyl-group-containing diamine compound No. 1, taken by use of a KBr tablet, is shown in FIG. 14.

#### 60 Example 1-1

[Synthesis of aromatic polycarbonate resin No. 1]

1.97 g (0.0023 mol) of N',N',N'',N''-tetra(4-methylphenyl)-1,4-bis[ $\alpha$ -(4-hydroxyphenyl)styryl]benzene-4',4"-diamine obtained in Preparation Example 1, represented by formula (4), and 0.70 g (0.0069 mol) of triethylamine were dissolved in 30 ml of dry tetrahydrofuran to prepare a solution (a). A solution (b) prepared by dissolving 0.558 g (0.0024 mol) of

diethylene glycol bis(chloroformate) in 5 ml of dry tetrahydrofuran was added dropwise to the solution (a) over a period of 30 minutes under water-cooled condition.

After completion of the addition, the resultant viscous reaction mixture was stirred for 90 minutes, and then 0.4 g of a dry tetrahydrofuran solution containing 4 wt. % of phenol was added to the reaction mixture, followed by stirring for 60 minutes.

Thereafter, the thus obtained viscous reaction mixture was caused to precipitate in methanol, and a crude product was separated from the reaction mixture by filtration. The product thus obtained was purified by repeating the process of dissolving the product in tetrahydrofuran and precipitating it in methanol twice. Thereafter, the precipitated product was filtered off, and dried, so that 2.14 g of an aromatic polycarbonate resin No. 1 according to the present invention having a repeat unit of the following formula was obtained in a yield of 91.48%.

[Aromatic polycarbonate resin No. 1]



The glass transition temperature ( $T_g$ ) of the above obtained aromatic polycarbonate resin No. 1 was 145.7° C.

The polystyrene-reduced number-average molecular weight and weight-average molecular weight, which were measured by the gel permeation chromatography, were respectively 15,900 and 82,000.

The results of the elemental analysis of the thus obtained compound are as follows:

| Elemental analysis: |       |      |      |
|---------------------|-------|------|------|
|                     | % C   | % H  | % N  |
| Found               | 80.39 | 5.71 | 2.85 |
| Calcd.              | 80.45 | 5.76 | 2.76 |

FIG. 7 shows an infrared spectrum of the aromatic polycarbonate resin No. 1, taken by use of KBr tablet.

The IR spectrum indicates the appearance of the characteristic absorption peak due to  $C=O$  stretching vibration of carbonate at  $1760\text{ cm}^{-1}$ .

### Example 1-2

#### [Synthesis of aromatic polycarbonate resin No. 2]

1.97 g (0.0023 mol) of  $N',N'',N''\text{-tetra}(4\text{-methylphenyl})-1,4\text{-bis}[\alpha\text{-(4-hydroxyphenyl)}\text{styryl}]benzene-4',4''\text{-diamine}$  obtained in Preparation Example 1, represented by formula (4), and 0.70 g (0.0069 mol) of triethylamine were dissolved in 40 ml of dry tetrahydrofuran to prepare a solution (a). A solution (b) prepared by dissolving 0.88 g (0.0024 mol) of polytetramethylene ether glycol bis(chloroformate), which was prepared from polytetramethylene ether glycol with an average molecular weight of 250, in 5 ml of dry tetrahydrofuran was added dropwise to the solution (a) over a period of 60 minutes under water-cooled condition.

After completion of the addition, the resultant viscous reaction mixture was stirred for 80 minutes, and then 0.4 g of a dry tetrahydrofuran solution containing 4 wt. % of phenol was added to the reaction mixture, followed by stirring for 60 minutes.

Thereafter, the thus obtained viscous reaction mixture was caused to precipitate in methanol, and a crude product was separated from the reaction mixture by filtration. The product thus obtained was purified by repeating the process of dissolving the product in tetrahydrofuran and precipitating it in methanol twice. Thereafter, the precipitated product was filtered off and dried, so that 2.24 g of an aromatic polycarbonate resin No. 2 according to the present invention having a repeat unit of the following formula was obtained in a yield of 84.68%.

[Aromatic polycarbonate resin No. 2]



The glass transition temperature ( $T_g$ ) of the above obtained aromatic polycarbonate resin No. 2 was 93.0°C.

The poly styrene-reduced number-average molecular weight and weight-average molecular weight, which were measured by the gel permeation chromatography, were respectively 10,494 and 28,811.

The results of the elemental analysis of the thus obtained compound are as follows:

| Elemental analysis: |       |      |
|---------------------|-------|------|
| % C                 | % H   | % N  |
| Found               | 79.44 | 6.69 |
| Calcd.              | 79.76 | 6.55 |

FIG. 8 shows an infrared spectrum of the aromatic polycarbonate resin No. 2, taken by use of KBr tablet.

The IR spectrum indicates the appearance of the characteristic absorption peak due to  $C=O$  stretching vibration of carbonate at  $1760\text{cm}^{-1}$ .

#### Example 1-3

[Synthesis of aromatic polycarbonate resin No. 3]

1.97 g (0.0023 mol) of  $N,N',N'',N''$ -tetra(4-methylphenyl)-1,4-bis[ $\alpha$ -(4-hydroxyphenyl)styryl]benzene-4',4"-diamine

25 obtained in Preparation Example 1, represented by formula (4), and 0.70 g (0.0069 mol) of triethylamine were dissolved in 40 ml of dry tetrahydrofuran to prepare a solution (a). A solution (b) prepared by dissolving 0.60 g (0.0025 mol) of 30 1,6-hexanediol bis(chloroformate) in 5 ml of dry tetrahydrofuran was added dropwise to the solution (a) over a period of 60 minutes under water-cooled condition.

35 After completion of the addition, the resultant viscous reaction mixture was stirred for 150 minutes, and then 0.4 g of a dry tetrahydrofuran solution containing 4 wt. % of phenol was added to the reaction mixture, followed by stirring for 60 minutes.

40 Thereafter, the thus obtained viscous reaction mixture was caused to precipitate in methanol, and a crude product was separated from the reaction mixture by filtration. The product thus obtained was purified by repeating the process of dissolving the product in tetrahydrofuran and precipitating it 45 in methanol twice. Thereafter, the precipitated product was filtered off and dried, so that 2.10 g of an aromatic polycarbonate resin No. 3 according to the present invention having a repeat unit of the following formula was obtained in a yield of 89.0%.

[Aromatic polycarbonate resin No. 3]



The glass transition temperature ( $T_g$ ) of the above obtained aromatic polycarbonate resin No. 3 was  $140.6^\circ C$ .

The polystyrene-reduced number-average molecular weight and weight-average molecular weight, which were measured by the gel permeation chromatography, were respectively 11,524 and 39,161.

The results of the elemental analysis of the thus obtained compound are as follows:

| Elemental analysis: |       |      |      |
|---------------------|-------|------|------|
|                     | % C   | % H  | % N  |
| Found               | 81.50 | 6.04 | 2.77 |
| Calcd.              | 81.85 | 6.08 | 2.73 |

FIG. 9 shows an infrared spectrum of the aromatic polycarbonate resin No. 3, taken by use of KBr tablet.

The IR spectrum indicates the appearance of the characteristic absorption peak due to  $C=O$  stretching vibration of carbonate at  $1760\text{cm}^{-1}$ .

#### Example 1-4

[Synthesis of aromatic polycarbonate resin No. 3']

4.71 g (0.0055 mol) of  $N,N',N'',N'''$ -tetra(4-methylphenyl)-1,4-bis[ $\alpha$ -(4-hydroxyphenyl)styryl]benzene-4',4"-diamine obtained in Preparation Example 1, represented by formula (4), and 1.67 g (0.0165 mol) of triethylamine were dissolved in 30 ml of dry tetrahydrofuran to prepare a solution (a). A solution (b) prepared by dissolving 1.44 g (0.0059 mol) of 1,6-hexanediol bis(chloroformate) in 8 ml of dry tetrahydrofuran was added dropwise to the solution (a) over a period of 60 minutes under water-cooled condition.

After completion of the addition, the resultant viscous reaction mixture was stirred for 24 hours, and then 0.8 g of a dry tetrahydrofuran solution containing 4 wt. % of phenol was added to the reaction mixture, followed by stirring for 60 minutes.

Thereafter, the thus obtained viscous reaction mixture was successively washed with a 5% aqueous solution of sodium hydroxide, a 2% aqueous solution of hydrochloric acid, and ion-exchange water, and then reprecipitated with methanol. Thus, a crude product was separated from the reaction

25 mixture by filtration, and dried, so that 5.03 g of an aromatic polycarbonate resin No. 3' according to the present invention having the same repeat unit as shown in Example 1-3 was obtained in a yield of 89.0%.

30 The glass transition temperature ( $T_g$ ) of the above obtained aromatic polycarbonate resin No. 3' was  $148.4^\circ C$ .

The polystyrene-reduced number-average molecular weight and weight-average molecular weight, which were measured by the gel permeation chromatography, were respectively 21,500 and 73,100.

35 The results of the elemental analysis of the thus obtained compound are as follows:

| Elemental analysis: |       |      |      |
|---------------------|-------|------|------|
|                     | % C   | % H  | % N  |
| Found               | 81.47 | 6.07 | 2.51 |
| Calcd.              | 81.85 | 6.08 | 2.73 |

40 FIG. 10 shows an infrared spectrum of the aromatic polycarbonate resin No. 3', taken by use of an NaCl film.

The IR spectrum indicates the appearance of the characteristic absorption peak due to  $C=O$  stretching vibration of carbonate at  $1760\text{cm}^{-1}$ .

#### Example 1-5

[Synthesis of aromatic polycarbonate resin No. 4]

1.71 g (0.002 mol) of  $N,N',N'',N'''$ -tetra(4-methylphenyl)-1,4-bis[ $\alpha$ -(4-hydroxyphenyl)styryl]benzene-4',4"-diamine obtained in Preparation Example 1, represented by formula (4) was dissolved in 30 ml of dry pyridine to prepare a solution (a). A solution (b) prepared by dissolving 0.356 g of triphosgene in 10 ml of dry pyridine was added dropwise to the solution (a) over a period of 30 minutes under water-cooled condition. Then, the thus obtained reaction mixture was stirred at  $17^\circ C$ . for 2 hours, and further stirred at  $30^\circ C$ . for one hour. With the addition of 30 mg of t-butylphenol to the above-mentioned reaction mixture, the mixture was stirred for one hour.

45 60 65 Thereafter, the resultant viscous reaction mixture was successively washed with a 5% aqueous solution of sodium hydroxide, a 2% aqueous solution of hydrochloric acid, and

33

ion-exchange water, and then reprecipitated with methanol. The resultant precipitated product was separated by filtration, and dried, so that 1.48 g of an aromatic polycarbonate resin No. 4 according to the present invention having a repeat unit of the following formula was obtained in a yield of 85.1%.

[Aromatic polycarbonate resin No. 4]



The glass transition temperature ( $T_g$ ) of the above obtained aromatic polycarbonate resin No. 4 was 196.7°C.

The polystyrene-reduced number-average molecular weight and weight-average molecular weight, which were measured by the gel permeation chromatography, were respectively 6,100 and 39,000.

The results of the elemental analysis of the thus obtained compound are as follows:

| Elemental analysis: |       |      |
|---------------------|-------|------|
| % C                 | % H   | % N  |
| Found               | 85.58 | 5.65 |
| Calcd.              | 85.69 | 5.71 |

FIG. 11 shows an infrared spectrum of the aromatic polycarbonate resin No. 4, taken by use of an NaCl film.

The IR spectrum indicates the appearance of the characteristic absorption peak due to  $\text{C}=\text{O}$  stretching vibration of carbonate at  $1780 \text{ cm}^{-1}$ .

#### Example 1-6

[Synthesis of aromatic polycarbonate resin No. 4']

1.71 g (0.002 mol) of  $\text{N}',\text{N}',\text{N}'',\text{N}''\text{-tetra(4-methylphenyl)}$ -1,4-bis[ $\alpha$ -(4-hydroxyphenyl)styryl]benzene-4',4"-diamine obtained in Preparation Example 1, represented by formula (4) was dissolved in a mixed solvent consisting of 10 ml of dry pyridine and 25 ml of methylene chloride to prepare a solution (a). A solution (b) prepared by dissolving 0.356 g of triphosgene in 10 ml of dry pyridine was added dropwise to the solution (a) over a period of 30 minutes under water-cooled condition. Then, the thus obtained reaction mixture was stirred at 17°C. for 2 hours. With the addition of 30 mg of t-butylphenol to the above-mentioned reaction mixture, the mixture was stirred for one hour.

Thereafter, the resultant viscous reaction mixture was reprecipitated with methanol, and a resultant precipitated product was separated by filtration and dried, so that 1.09 g of an aromatic polycarbonate resin No. 4' according to the present invention having the same repeat unit as shown in Example 1-5 was obtained in a yield of 62.5%.

The polystyrene-reduced number-average molecular weight and weight-average molecular weight, which were

34

measured by the gel permeation chromatography, were respectively 6,700 and 64,700.

The IR spectrum of the aromatic polycarbonate resin No. 4' indicates the appearance of the characteristic absorption peak due to  $\text{C}=\text{O}$  stretching vibration of carbonate at  $1780 \text{ cm}^{-1}$ .

#### Example 1-7

[Synthesis of aromatic polycarbonate resin No. 4"]

1.71 g (0.002 mol) of  $\text{N}',\text{N}',\text{N}'',\text{N}''\text{-tetra(4-methylphenyl)}$ -1,4-bis[ $\alpha$ -(4-hydroxyphenyl)styryl]benzene-4',4"-diamine obtained in Preparation Example 1, represented by formula (4) was placed into a reaction vessel. An aqueous solution prepared by dissolving 0.32 g (0.008 mol) of sodium hydroxide in 30 ml of ion-exchange water was added to the above-mentioned dihydroxyl-group-containing diamine compound No. 1, and a mixture thus obtained was stirred. A solution prepared by dissolving 0.356 g (0.0012 mol) of triphosgene in 10 ml of methylene chloride was added dropwise to the above-mentioned mixture over a period of 20 minutes under ice-cooled condition.

Furthermore, 5 ml of methylene chloride was added to the reaction mixture as rinsing the vessel. Then, 0.1 g (0.025 mol) of sodium hydroxide was added to the reaction mixture at room temperature. Further, with the addition of one drop of triethylamine, the reaction mixture was stirred for 3 hours.

Thereafter, the resultant viscous reaction mixture was successively washed with a 5% aqueous solution of sodium hydroxide, a 2% aqueous solution of hydrochloric acid, and ion-exchange water, and reprecipitated with methanol. The resultant precipitate was separated from the reaction mixture by filtration, and dried, so that 1.35 g of an aromatic polycarbonate resin No. 4" according to the present invention having the same repeat unit as shown in Example 1-5 was obtained in a yield of 77.6%.

The polystyrene-reduced number-average molecular weight and weight-average molecular weight, which were measured by the gel permeation chromatography, were respectively 4,500 and 102,000.

The results of the elemental analysis of the thus obtained compound are as follows:

| Elemental analysis: |       |      |
|---------------------|-------|------|
| % C                 | % H   | % N  |
| Found               | 85.89 | 5.69 |
| Calcd.              | 85.69 | 5.71 |

The IR spectrum of the aromatic polycarbonate resin No. 4" indicates the appearance of the characteristic absorption peak due to  $\text{C}=\text{O}$  stretching vibration of carbonate at  $1780 \text{ cm}^{-1}$ .

#### Example 1-8

[Synthesis of aromatic polycarbonate resin No. 4'"]

1.71 g (0.002 mol) of  $\text{N}',\text{N}',\text{N}'',\text{N}''\text{-tetra(4-methylphenyl)}$ -1,4-bis[ $\alpha$ -(4-hydroxyphenyl)styryl]benzene-4',4"-diamine obtained in Preparation Example 1, represented by formula (4) was placed into a reaction vessel. An aqueous solution prepared by dissolving 0.32 g (0.008 mol) of sodium hydroxide in 200 ml of ion-exchange water was added to the above-mentioned dihydroxyl-group-containing diamine compound No. 1, and a mixture thus obtained was stirred. A solution prepared by dissolving 0.356 g (0.0012 mol) of triphosgene in 130 ml of methylene chloride was added dropwise to the above-mentioned mixture over a period of 20 minutes under ice-cooled condition.

## 35

Furthermore, 20 ml of methylene chloride was added to the reaction mixture as rinsing the vessel. Then, 0.1 g (0.025 mol) of sodium hydroxide was added to the reaction mixture at room temperature. Further, with the addition of one drop of triethylamine, the reaction mixture was stirred for 3 hours.

Thereafter, the resultant viscous reaction mixture was successively washed with a 5% aqueous solution of sodium hydroxide, a 2% aqueous solution of hydrochloric acid, and ion-exchange water, and reprecipitated with methanol. The resultant precipitate was separated from the reaction mixture by filtration, and dried, so that 1.30 g of an aromatic polycarbonate resin No. 4" according to the present invention having the same repeat unit as shown in Example 1-5 was obtained in a yield of 74.6%.

The glass transition temperature ( $T_g$ ) of the above obtained aromatic polycarbonate resin No. 4" was 198.8°C.

The polystyrene-reduced number-average molecular weight and weight-average molecular weight, which were measured by the gel permeation chromatography, were respectively 16,700 and 116,000.

The results of the elemental analysis of the thus obtained compound are as follows:

| Elemental analysis: |       |      |
|---------------------|-------|------|
| % C                 | % H   | % N  |
| Found               | 85.58 | 5.66 |
| Calcd.              | 85.69 | 5.71 |

The IR spectrum of the aromatic polycarbonate resin No. 4" indicates the appearance of the characteristic absorption peak due to  $\text{C}=\text{O}$  stretching vibration of carbonate at 1780  $\text{cm}^{-1}$ .

## Example 1-9

## [Synthesis of aromatic polycarbonate resin No. 5]

3.86 g (0.0045 mol) of  $\text{N}^{\prime},\text{N}^{\prime\prime},\text{N}^{\prime\prime\prime},\text{N}^{\prime\prime\prime\prime}$ -tetra(4-methylphenyl)-1,4-bis[ $\alpha$ -(4-hydroxyphenyl)styryl]benzene-4',4"-diamine obtained in Preparation Example 1, represented by formula (4), and 1.02 g (0.0045 mol) of bisphenol A were placed into a reaction vessel.

An aqueous solution prepared by dissolving 1.44 g (0.036 mol) of sodium hydroxide and 0.015 g of sodium hydrosulfide in 60 ml of ion-exchange water was added to the above-mentioned mixture in the reaction vessel, and a mixture thus obtained was stirred at 65°C. for several minutes. Then, with the addition of 0.45 g of sodium hydroxide, the reaction mixture was stirred. Furthermore, an aqueous solution prepared by dissolving 1.44 g (0.036 mol) of sodium hydroxide and 0.015 g of sodium hydrosulfide in 60 ml of ion-exchange water was again added to the above-mentioned mixture, and a mixture thus obtained was stirred at room temperature.

With the addition of 30 ml of tetrahydrofuran, the above-mentioned mixture was vigorously stirred. Then, a solution prepared by dissolving 1.61 g (0.0054 mol) of triphosgene in 50 ml of methylene chloride was added dropwise to the above-mentioned mixture over a period of 20 minutes under ice-cooled condition.

Thereafter, with the addition of one drop of triethylamine, the reaction mixture was further stirred for 2 hours. Further, the reaction mixture was stirred for 30 minutes with the addition thereto of 135 mg of tert-butylphenol.

The resultant viscous reaction mixture was successively washed with a 5% aqueous solution of sodium hydroxide, a

## 36

2% aqueous solution of hydrochloric acid, and ion-exchange water, and reprecipitated with methanol. The reaction product was separated by filtration, and dried, so that 4.45 g of an aromatic polycarbonate resin No. 5 according to the present invention having a repeat unit of the following formula was obtained in a yield of 86.9%.

[Aromatic polycarbonate resin No. 5]



The glass transition temperature ( $T_g$ ) of the above obtained aromatic poly carbonate resin No. 5 was 183.0°C.

The polystyrene-reduced number-average molecular weight and weight-average molecular weight, which were measured by the gel permeation chromatography, were respectively 10,600 and 44,200.

The results of the elemental analysis of the thus obtained compound are as follows:

| Elemental analysis: |       |      |
|---------------------|-------|------|
| % C                 | % H   | % N  |
| Found               | 84.38 | 5.60 |
| Calcd.              | 83.41 | 5.68 |

FIG. 12 shows an infrared spectrum of the aromatic polycarbonate resin No. 5, taken by use of an NaCl film.

The IR spectrum of the aromatic polycarbonate resin No. 5 indicates the appearance of the characteristic absorption peak due to  $\text{C}=\text{O}$  stretching vibration of carbonate at 1775  $\text{cm}^{-1}$ .

## Example 1-10

## [Synthesis of aromatic polycarbonate resin No. 5]

3.42 g (0.004 mol) of  $\text{N}^{\prime},\text{N}^{\prime\prime},\text{N}^{\prime\prime\prime},\text{N}^{\prime\prime\prime\prime}$ -tetra(4-methylphenyl)-1,4-bis[ $\alpha$ -(4-hydroxyphenyl)styryl]benzene-4',4"-diamine obtained in Preparation Example 1, represented by formula (4), and 0.91 g (0.004 mol) of bisphenol A were placed into a reaction vessel.

An aqueous solution prepared by dissolving 1.28 g (0.032 mol) of sodium hydroxide in 800 ml of ion-exchange water was added to the above-mentioned mixture in the reaction vessel, and a mixture thus obtained was stirred.

Then, a solution prepared by dissolving 1.42 g (0.0048 mol) of triphosgene in 500 ml of methylene chloride was added dropwise to the above-mentioned mixture over a period of 20 minutes under ice-cooled condition. Thereafter, 100 ml of methylene chloride was added to the reaction

37

mixture with rinsing the reaction vessel, and 0.4 g of sodium hydroxide was further added at room temperature. Then, with the addition of one drop of triethylamine, the reaction mixture was further stirred for 3 hours.



The resultant viscous reaction mixture was successively washed with a 5% aqueous solution of sodium hydroxide, a 2% aqueous solution of hydrochloric acid, and ion-exchange water, and reprecipitated with methanol. The reaction product was separated by filtration, and dried, so that 3.36 g of an aromatic polycarbonate resin No. 5' according to the present invention having the same repeat unit as shown in Example 1-9 was obtained in a yield of 74.1%.

The glass transition temperature ( $T_g$ ) of the above obtained aromatic polycarbonate resin No. 5' was 189.3°C.

The polystyrene-reduced number-average molecular weight and weight-average molecular weight, which were measured by the gel permeation chromatography, were respectively 15,600 and 76,300.

The results of the elemental analysis of the thus obtained compound are as follows:

Elemental analysis:

|        | % C   | % H  | % N  | 40 |
|--------|-------|------|------|----|
| Found  | 83.10 | 5.59 | 2.17 |    |
| Calcd. | 83.41 | 5.68 | 2.46 |    |

The IR spectrum of the aromatic polycarbonate resin No. 5' indicates the appearance of the characteristic absorption peak due to C=O stretching vibration of carbonate at 1775  $\text{cm}^{-1}$ .

**Example 2-1**

[Fabrication of Photoconductor No. 1]  
(Formation of intermediate layer)

A commercially available polyamide resin (Trademark "CM-8000", made by Toray Industries, Inc.) was dissolved in a mixed solvent of methanol and butanol, so that a coating liquid for an intermediate layer was prepared.

The thus prepared coating liquid was coated on an aluminum plate by a doctor blade, and dried at room temperature, so that an intermediate layer with a thickness of 0.3  $\mu\text{m}$  was provided on the aluminum plate.

(Formation of charge generation layer)

A coating liquid for a charge generation layer was prepared by dispersing a bisazo compound of the following formula (hereinafter referred to as "Pig 1"), serving as a charge generation material, in a mixed solvent of cyclohexanone and methyl ethyl ketone in a ball mill. The thus obtained coating liquid was coated on the above prepared intermediate layer by a doctor blade, and dried at room

38

temperature. Thus, a charge generation layer with a thickness of about 1  $\mu\text{m}$  was formed on the intermediate layer.

[Bisazo compound (Pig. 1)]



20 (Formation of charge transport layer)

The aromatic polycarbonate resin No. 1 of the present invention prepared in Example 1-1, serving as a charge transport material, was dissolved in dichloromethane. The thus obtained coating liquid was coated on the above prepared charge generation layer by a doctor blade, and dried at room temperature and then at 120°C. for 20 minutes, so that 25 a charge transport layer with a thickness of about 20  $\mu\text{m}$  was provided on the charge generation layer.

30 Thus, an electrophotographic photoconductor No. 1 according to the present invention was fabricated.

**Examples 2-2 to 2-5**

40 The procedure for fabrication of the electrophotographic photoconductor No. 1 in Example 2-1 was repeated except that the aromatic polycarbonate resin No. 1 for use in the 45 charge transport layer coating liquid in Example 2-1 was replaced by each of the aromatic polycarbonate resins (as illustrated in Table 1).

50 Thus, electrophotographic photoconductors No. 2 to No. 5 according to the present invention were fabricated.

**Examples 2-6**

55 The procedure for fabrication of the electrophotographic photoconductor No. 2 in Example 2-2 was repeated except that the bisazo compound "Pig. 1" for use in the charge generation layer coating liquid in Example 2-2 was replaced by a trisazo compound (hereinafter referred to as "Pig. 2.") 60 of the following formula:

[Trisazo compound (Pig. 2)]



Thus, an electrophotographic photoconductor No. 6 according to the present invention was fabricated.

## Example 2-7

The procedure for fabrication of the electrophotographic photoconductor No. 6 in Example 2-6 was repeated except that the aromatic polycarbonate resin No. 2 for use in the charge transport layer coating liquid in Example 2-6 was replaced by the aromatic polycarbonate resin No. 3 prepared in Example 1-3.

Thus, an electrophotographic photoconductor No. 7 according to the present invention was fabricated.

Each of the electrophotographic photoconductors No. 1 through No. 7 according to the present invention obtained in Examples 2-1 to 2-7 was charged negatively in the dark under application of -6 kV of corona charge for 20 seconds, using a commercially available electrostatic copying sheet testing apparatus ("Paper Analyzer Model SP-428" made by Kawaguchi Electro Works Co., Ltd.). Then, each electrophotographic photoconductor was allowed to stand in the dark for 20 seconds without applying any charge thereto, and the surface potential  $V_o$  (V) of the photoconductor was measured. Each photoconductor was then illuminated by a tungsten lamp in such a manner that the illuminance on the illuminated surface of the photoconductor was 4.5 lux, and the exposure  $E_{1/2}$  (lux.sec) required to reduce the initial surface potential  $V_o$  (V) to  $\frac{1}{2}$  the initial surface potential  $V_o$  (V) was measured. The results are shown in Table 1.

TABLE 1

| Example No. | CGM   | Aromatic Polycarbonate Resin No. | $-V_o$ (V) | $E_{1/2}$ (lux.sec) |
|-------------|-------|----------------------------------|------------|---------------------|
| 2-1         | Pig.1 | No. 1                            | 905        | 0.78                |
| 2-2         | Pig.1 | No. 2                            | 988        | 0.65                |
| 2-3         | Pig.1 | No. 3                            | 1190       | 0.67                |
| 2-4         | Pig.1 | No. 4                            | 667        | 0.66                |
| 2-5         | Pig.1 | No. 5                            | 782        | 0.75                |
| 2-6         | Pig.2 | No. 2                            | 441        | 0.30                |
| 2-7         | Pig.2 | No. 3                            | 505        | 0.37                |

Furthermore, each of the above obtained electrophotographic photoconductors No. 1 to No. 7 was set in a commercially available electrophotographic copying machine, and the photoconductor was charged and exposed to light images via the original images to form latent electrostatic images thereon. Then, the latent electrostatic images formed on the photoconductor were developed into

visible toner images by a dry developer, and the visible toner images were transferred to a sheet of plain paper and fixed thereon. As a result, clear toner images were obtained on the paper. When a wet developer was employed for the image formation, clear images were formed on the paper similarly.

As previously explained, the polycarbonate resin for use in the photoconductive layer of the electrophotographic photoconductor according to the present invention comprises a repeat unit of formula (I); or repeat units of formulae (II) and (III). Any of the above-mentioned aromatic polycarbonate resins have the charge transporting properties and high mechanical strength, so that the photosensitivity and durability of the photoconductor are sufficiently high.

Japanese Patent Application No. 7-330479 filed Dec. 19, 1995; Japanese Patent Application No. 8-009408 filed Jan. 23, 1996; Japanese Patent Application No. 8-014098 filed Jan. 30, 1996; Japanese Patent Application No. 8-336002 filed Dec. 16, 1996; and Japanese Patent Application No. 8-338295 filed Dec. 18, 1996 are hereby incorporated by reference.

What is claimed is:

1. An electrophotographic photoconductor comprising an electroconductive support, and a photoconductive layer formed thereon comprising as an effective component an aromatic polycarbonate resin having a repeat unit of formula (I):



wherein n is an integer of 5 to 5000; Ar<sup>3</sup> and Ar<sup>4</sup> may be the same or different, and is a bivalent aromatic hydrocarbon group which may have a substituent or a bivalent heterocyclic group which may have a substituent; Ar<sup>1</sup>, Ar<sup>2</sup>, Ar<sup>5</sup> and Ar<sup>6</sup> each may be the same or different, and is an aromatic hydrocarbon group which may have a substituent, or a heterocyclic group which may have a substituent; and X is a bivalent aliphatic group, a bivalent cyclic aliphatic group, or



in which R<sup>1</sup> and R<sup>2</sup> are each independently an alkyl group which may have a substituent, an aromatic hydrocarbon group which may have a substituent, or a halogen atom; l and m are each independently an integer of 0 to 4; and p is an integer of 0 or 1, and when p=1, Y is a straight-chain, branched or cyclic alkylene group having 1 to 12 carbon atoms,



-continued

or



in which Z is a bivalent aliphatic hydrocarbon group; a is an integer of 0 to 20; b is an integer of 1 to 2000; and R<sup>3</sup> and R<sup>4</sup> are each independently an alkyl group which may have a substituent or an aromatic hydrocarbon group which may have a substituent.

2. The electrophotographic photoconductor as claimed in claim 1, wherein said bivalent aromatic hydrocarbon group represented by Ar<sup>3</sup> and Ar<sup>4</sup> is phenylene group.

3. An electrophotographic photoconductor comprising an electroconductive support, and a photoconductive layer formed thereon comprising as an effective component an aromatic polycarbonate resin having a repeat unit of formula (II) and a repeat unit of formula (III), with the composition ratio of the repeat unit of formula (II) to the repeat unit of formula (III) being in the relationship of 0<k/(k+j)≤1:



wherein k is an integer of 5 to 5000; j is an integer of 0 to 5000; Ar<sup>3</sup> and Ar<sup>4</sup> may be the same or different, and is a bivalent aromatic hydrocarbon group which may have a substituent or a bivalent heterocyclic group which may have a substituent; Ar<sup>1</sup>, Ar<sup>2</sup>, Ar<sup>5</sup> and Ar<sup>6</sup> each may be the same or different, and is an aromatic hydrocarbon group which may have a substituent, or a heterocyclic group which may have a substituent; and X is a bivalent aliphatic group, a bivalent cyclic aliphatic group, or



in which R<sup>1</sup> and R<sup>2</sup> are each independently an alkyl group which may have a substituent, an aromatic hydrocarbon group which may have a substituent, or a halogen atom; i and m are each independently an integer of 0 to 4; and p is an integer of 0 or 1, and when p=1, Y is a straight-chain, branched or cyclic alkylene group having 1 to 12 carbon atoms,



in which Z is a bivalent aliphatic hydrocarbon group; a is an integer of 0 to 20; b is an integer of 1 to 2000; and R<sup>3</sup> and R<sup>4</sup> are each independently an alkyl group which may have a substituent or an aromatic hydrocarbon group which may have a substituent.

4. The electrophotographic photoconductor as claimed in claim 3, wherein said bivalent aromatic hydrocarbon group represented by Ar<sup>3</sup> and Ar<sup>4</sup> is phenylene group.

5. The electrophotographic photoconductor as claimed in claim 1, wherein said bivalent aromatic hydrocarbon group represented by Ar<sup>3</sup> and Ar<sup>4</sup> is a bivalent group derived from

40 one aromatic hydrocarbon group selected from the group consisting of benzene, naphthalene, biphenyl, terphenyl, pyrene, fluorene, and 9,9-dimethylfluorene.

45 6. The electrophotographic photoconductor as claimed in claim 1, wherein said bivalent heterocyclic group represented by Ar<sup>3</sup> and Ar<sup>4</sup> is a bivalent group derived from one heterocyclic group selected from the group consisting of thiophene, benzothiophene, furan, benzofuran and carbazole.

50 7. The electrophotographic photoconductor as claimed in claim 1, wherein said bivalent heterocyclic group represented by Ar<sup>3</sup> and Ar<sup>4</sup> is diphenyl ether group in which two aryl groups are bonded via oxygen, or diphenyl thioether group in which two aryl groups are bonded via sulfur.

55 8. The electrophotographic photoconductor as claimed in claim 1, wherein said substituent for said bivalent aromatic hydrocarbon group and said bivalent heterocyclic group represented by Ar<sup>3</sup> and Ar<sup>4</sup> is selected from the group consisting of a halogen atom, cyano group, nitro group, an alkyl group having 1 to 12 carbon atoms, an alkoxy group having 1 to 12 carbon atoms, an aryloxy group, a substituted mercapto group, an arylmercapto group, an alkyl-substituted amino group, and an acyl group.

60 9. The electrophotographic photoconductor as claimed in claim 1, wherein said aromatic hydrocarbon group represented by Ar<sup>1</sup>, Ar<sup>2</sup>, Ar<sup>5</sup> and Ar<sup>6</sup> is an aromatic hydrocarbon

group selected from the group consisting of phenyl group, naphthyl group, biphenyl group, terphenyl group, pyrenyl group, fluorenyl group, and 9,9-dimethyl-2-fluorenyl group.

10. The electrophotographic photoconductor as claimed in claim 1, wherein said heterocyclic group represented by  $Ar^1$ ,  $Ar^2$ ,  $Ar^5$  and  $Ar^6$  is a heterocyclic group selected from the group consisting of thieryl group, benzothienyl group, furyl group, benzofuranyl group and carbazolyl group.

11. The electrophotographic photoconductor as claimed in claim 1, wherein said substituent for said aromatic hydrocarbon group and said heterocyclic group represented by  $Ar^1$ ,  $Ar^2$ ,  $Ar^3$  and  $Ar^4$  is selected from the group consisting of a halogen atom, cyano group, nitro group, an alkyl group having 1 to 12 carbon atoms, an alkoxy group having 1 to 12 carbon atoms, an aryloxy group, a substituted mercapto group, an arylmercapto group, an alkyl-substituted amino group, and an acyl group.

12. The electrophotographic photoconductor as claimed in claim 1, wherein said aromatic hydrocarbon group represented by  $R^1$  to  $R^4$  is selected from the group consisting of phenyl group which may have a substituent, and biphenyl group which may have a substituent.

13. The electrophotographic photoconductor as claimed in claim 1, wherein said alkyl group represented by  $R^1$  to  $R^4$  has 1 to 12 carbon atoms.

14. The electrophotographic photoconductor as claimed in claim 3, wherein said bivalent aromatic hydrocarbon group represented by  $Ar^3$  and  $Ar^4$  is a bivalent group derived from one aromatic hydrocarbon group selected from the group consisting of benzene, naphthalene, biphenyl, terphenyl, pyrene, fluorene, and 9,9-dimethylfluorene.

15. The electrophotographic photoconductor as claimed in claim 3, wherein said bivalent heterocyclic group represented by  $Ar^3$  and  $Ar^4$  is a bivalent group derived from one heterocyclic group selected from the group consisting of thiophene, benzothiophene, furan, benzofuran and carbazole.

16. The electrophotographic photoconductor as claimed in claim 3, wherein said bivalent heterocyclic group repre-

sented by  $Ar^3$  and  $Ar^4$  is diphenyl ether group in which two aryl groups are bonded via oxygen, or diphenyl thioether group in which two aryl groups are bonded via sulfur.

17. The electrophotographic photoconductor as claimed in claim 3, wherein said substituent for said bivalent aromatic hydrocarbon group and said bivalent heterocyclic group represented by  $Ar^3$  and  $Ar^4$  is selected from the group consisting of a halogen atom, cyano group, nitro group, an alkyl group having 1 to 12 carbon atoms, an alkoxy group having 1 to 12 carbon atoms, an aryloxy group, a substituted mercapto group, an arylmercapto group, an alkyl-substituted amino group, and an acyl group.

18. The electrophotographic photoconductor as claimed in claim 3, wherein said aromatic hydrocarbon group represented by  $Ar^1$ ,  $Ar^2$ ,  $Ar^3$  and  $Ar^6$  is an aromatic hydrocarbon group selected from the group consisting of phenyl group, naphthyl group, biphenyl group, terphenyl group, pyrenyl group, fluorenyl group, and 9,9-dimethyl-2-fluorenyl group.

19. The electrophotographic photoconductor as claimed in claim 3, wherein said heterocyclic group represented by  $Ar^1$ ,  $Ar^2$ ,  $Ar^5$  and  $Ar^6$  is a heterocyclic group selected from the group consisting of thieryl group, benzothienyl group, furyl group, benzofuranyl group and carbazolyl group.

20. The electrophotographic photoconductor as claimed in claim 3, wherein said substituent for said aromatic hydrocarbon group and said heterocyclic group represented by  $Ar^1$ ,  $Ar^2$ ,  $Ar^5$  and  $Ar^6$  is selected from the group consisting of a halogen atom, cyano group, nitro group, an alkyl group having 1 to 12 carbon atoms, an alkoxy group having 1 to 12 carbon atoms, an aryloxy group, a substituted mercapto group, an arylmercapto group, an alkyl-substituted amino group, and an acyl group.

21. The electrophotographic photoconductor as claimed in claim 3, wherein said aromatic hydrocarbon group represented by  $R^1$  to  $R^4$  is selected from the group consisting of phenyl group which may have a substituent, and biphenyl group which may have a substituent.

22. The electrophotographic photoconductor as claimed in claim 3, wherein said alkyl group represented by  $R^1$  to  $R^4$  has 1 to 12 carbon atoms.

\* \* \* \* \*

UNITED STATES PATENT AND TRADEMARK OFFICE  
**CERTIFICATE OF CORRECTION**

PATENT NO. : 5,846,680

Page 1 of 2

DATED : December 8, 1998

INVENTOR(S) : Adachi, et al.

It is certified that error appears in the above-identified patent and that said Letters Patent is hereby corrected as shown below:

Column 3, line 54, change "Ar<sup>1</sup>, Ar<sup>2</sup>, Ar<sup>3</sup> and Ar<sup>4</sup>" to  
--Ar<sup>1</sup>, Ar<sup>2</sup>, Ar<sup>5</sup> and Ar<sup>6</sup>--.

Column 7, line 14, change "i s" to --is--.

Column 8, line 9, change "amino" to --amine--;  
line 61, change "poly carbonate" to --polycarbonate--.

Column 10, line 38, change "In" to --in--.

Column 15, line 35, change "amido" to --amide--;  
line 62, change "other" to --ether--.

Column 17, line 56, change "a s" to --as--.

UNITED STATES PATENT AND TRADEMARK OFFICE  
**CERTIFICATE OF CORRECTION**

PATENT NO. : 5,846,680  
DATED : December 8, 1998  
INVENTOR(S) : Adachi, et al.

Page 2 of 2

It is certified that error appears in the above-identified patent and that said Letters Patent is hereby corrected as shown below:

Column 23, line 1, change "photoconductor u" to --photoconductor--.

Column 40, line 62, change "-O-, -S-, -SO-, -SO<sub>3</sub>-" to  
-- -O-, -S-, -SO-, -SO<sub>2</sub> --.

Column 42, line 67, change "Ar<sup>2, Ar<sup>5</sup></sup>" to --Ar<sup>2</sup>, Ar<sup>5</sup>--.

Signed and Sealed this  
Ninth Day of January, 2001

Attest:



Q. TODD DICKINSON

Attesting Officer

Commissioner of Patents and Trademarks